

## UNITED STATES PATENT OFFICE.

CHARLES R. FRANKLIN, OF DOVER, NEW JERSEY.

## PROPELLENT POWDER.

No Drawing.

Application filed October 9, 1923. Serial No. 667,555.

(GRANTED UNDER THE ACT OF MARCH 3, 1883; 22 STAT. L. 625.)

*To all whom it may concern:*

Be it known that I, CHARLES R. FRANKLIN, a citizen of the United States, and a resident of Dover, county of Morris, and 5 State of New Jersey, have invented an Improvement in Propellant Powders, of which the following is a specification.

The invention described herein may be used by the Government, or any of its 10 officers or employees in prosecution of work for the Government, or by any other person in the United States, without payment to me of any royalty thereon, in accordance with the act of March 3, 1883.

15 The subject of the present invention is a propellant powder.

The primary object of my invention is the provision of a propellant powder which will be smokeless and flashless, non-hygroscopic 20 and which will meet all ballistic requirements.

A further object is the establishment of a method whereby a propellant powder having the qualities recited above may be manufactured in such way that it may be used immediately upon the completion of its manufacture without the necessity of drying the completed article.

With the foregoing and other objects in 30 view, my invention resides in the novel arrangement and combination of parts and in the details of construction hereinafter described and claimed, it being understood that changes in the precise embodiment of 35 the invention herein disclosed may be made within the scope of what is claimed without departing from the spirit of the invention.

A powder such as forms the subject of 40 my invention is preferably composed of nitrocellulose, nitroglycerin, a non-hygroscopic and deterrent material such as trinitrotoluol, a flash reducing agent such as hydrocellulose and a stabilizer such as diphenylamine.

45 Such a powder may be made according to the process described herein. Nitrocellulose of suitable solubility and having approximately 12.60% nitrogen content is first mixed with a large amount of water, approximately 6 to 10 times the weight of the nitrocotton. The mixture of the nitrocellulose and water has an appearance not unlike that of a flour batter. To this mixture is added the required amount of nitroglycerin 55 with violent agitation, the more violent the

agitation, the more uniformly will the nitroglycerine be distributed. The agitation is continued for a suitable period, which in practice has been found to be approximately 30 minutes after the last portion of the 60 nitroglycerine has been added. This portion of the process is designated in the manufacture as "wet mixing".

The mixture is then transferred to a centrifuge or other machine having a similar 65 function, and the excess water separated from the other ingredients by wringing. The moisture content of the solid material thus treated will range from 20% to 45%, 70 20% to 25% being preferable.

The material is then transferred to a dough mixing machine similar to that used for manufacture of U. S. Army Service powder. This machine is placed in operation and a suitable amount of trinitrotoluol or other organic body having similar 75 qualities is added. After a proper interval, which in practice has been found to be approximately 5 minutes, the necessary amount of hydrocellulose or other flame 80 reducing ingredient is added. This last named material may be added when in the wet or dried state. With the hydrocellulose or other flame reducing ingredient is also added a proper amount of a stabilizer such 85 as diphenylamine.

The last named is then mixed for 30 minutes after the addition of the last component. This process in the manufacture is 90 termed the first dry mixing.

The material is then passed through pressure rollers heated to a temperature of preferably 80° C. to 100° C. This step in the manufacture is known as the first preliminary rolling and represents a most important step in the process. During this 95 rolling the water content of the mass is reduced, the colloiding action of the nitroglycerine is promoted and the ingredients having a low melting point are brought into 100 more intimate contact with the other components.

The material as removed from the rollers at the end of this preliminary rolling is seasoned for a suitable period, generally 24 to 105 48 hours at a temperature of 50° C. to 60° C. During this step in the manufacture the water content is reduced to a negligible quantity and the material takes on a more or less flaky appearance.

The seasoned material is then, again, passed through pressure rollers heated to the proper temperature, in practice generally between 80° C. to 100° C., until it takes on the appearance of transparent amber, that is, it is a translucent, cohering, colloided solid, adhering closely to the pressure rolls. This step is designated as the second or final rolling.

10 The material is then cut from the rolls in the form of a tough, pliable sheet having the desired thickness, width and length. It is then cut or stamped in the shape desired and is ready for use.

15 The various ingredients which compose my powder may be mixed in widely varied proportions. A composition which has proven successful in practice is as follows: nitrocellulose, 49.5%; nitroglycerine, 20%; trinitrotoluol, 20%; hydrocellulose, 10%; diphenylamine, 5%. The composition and proportions cited herein are merely intended as an example of a powder which may be made by my process and which will have the

20 desired ballistic qualities. It is by no means intended to limit my invention to a formula such as given above. Variations of this formula within the scope of my invention will readily occur to those skilled in art.

25 For the trinitrotoluol any organic compound such as dinitrotoluol, trinitrobenzene, etc., having similar qualities may be substituted; starch or any other flame reducing agent may be substituted for the hydro-

30 cellulose while for the diphenylamine any amino compound, such as urea or aniline, or any compound having similar properties may be substituted.

This powder has been found especially useful in a 75 m/m. gun and other cannons, but it is by no means limited to such use.

A powder manufactured by the process that I have described and composed of ingredients such as described requires no drying and is therefore ready for use immediately after manufacture. This quality is largely due to the fact that the powder is manufactured without the use of a volatile solvent agent as ether-alcohol mixture, acetone, amylacetate, etc. Powder made with such solvents require a period of time often as great as 35 days to remove the volatile colloiding agent.

Furthermore, a powder made according to the process described and with constituents such as set forth is non-hygroscopic, whereas, the present U. S. Army Service powder is not. The powder then made according to my invention may be packed in ordinary packing cases, whereas, the service ammunition requires special air-tight cases; this for the reason that the regular U. S. Service powder has some of the volatile solvent, used in its manufacture, remaining in the powder, the amount depending upon

the caliber of the gun with which the powder is intended to be used. A powder manufactured by the method described and having constituents as set forth will be smokeless, flashless, non-hygroscopic, and, in practice, has been found to meet all ballistic requirements.

I claim:

1. A propellant powder containing approximately 49.5% nitrocellulose, 20% nitroglycerine, 20% trinitrotoluol, 10% hydrocellulose and .5% diphenylamine. 75
2. A propellant powder consisting of a stabilized mixture, of nitrocellulose, nitroglycerine, trinitrotoluol, and hydrocellulose. 80
3. A propellant powder containing nitrocellulose, nitroglycerine, trinitrotoluol, and hydrocellulose. 85
4. A propellant powder containing nitrocellulose, nitroglycerine, a non-hygroscopic agent and hydrocellulose. 90
5. A propellant powder containing nitrocellulose, nitroglycerine, a nitrohydrocarbon, and hydrocellulose. 95
6. A propellant powder containing nitrocellulose, nitroglycerine, a non-hygroscopic deterrent material and a flame reducing compound. 100
7. A propellant powder containing nitrocellulose, nitroglycerine, a nitrohydrocarbon and a flame reducing compound. 105
8. A propellant powder consisting of a stabilized mixture of nitrocellulose, nitroglycerine, trinitrotoluol, and a flame reducing compound. 110
9. A propellant powder consisting of a stabilized mixture of nitrocellulose, nitroglycerine, a deterrent material and hydrocellulose. 115
10. A propellant powder consisting of stabilized mixture of nitrocellulose, nitroglycerine, a non-hygroscopic agent, and hydrocellulose. 120
11. A process of preparing a propellant powder consisting in first mixing nitrocellulose of approximately 12.60% nitrogen content with a large excess of water until it has an appearance like that of a flour batter, then adding nitroglycerine with rapid agitation, then wringing out the excess of water, then adding a non-hygroscopic deterrent, then after an interval a flash reducing compound and a stabilizer, then mixing the whole together, then passing the mixed material through the heated pressure rolls, then seasoning, then again passing through heated pressure rolls until the material becomes a translucent cohering, colloided solid, and then cutting to the proper shapes and sizes. 125
12. The process of preparing a propellant powder consisting in first mixing nitrocellulose of suitable nitrogen content with a large excess of water, then adding nitroglycerine with rapid agitation, then wringing out the excess of water, then adding a non-hygroscopic agent and a flash reducing compound 130

and a stabilizer and mixing the whole together, then subjecting the material thus formed to pressure and heat, then seasoning the whole, then again subjecting the material to pressure and heat until the mass becomes a translucent, cohering, colloided solid, and then cutting into proper shapes and sizes.

13. The process of preparing a propellant powder consisting in first mixing nitrocellulose of suitable nitrogen content with a large excess of water, then adding nitroglycerine with rapid agitation, then wringing out the excess of water, then adding a nonhygroscopic agent, a flash reducing compound and a stabilizer, then mixing the whole, then subjecting the whole to pressure, then seasoning then again subjecting the whole to pres-

sure until the material becomes a translucent, cohering, colloided solid and then cutting into the proper shapes and sizes. 20

14. The process of preparing a propellant powder consisting in first mixing nitrocellulose of suitable nitrogen content with a large excess of water, then adding nitrogen with rapid agitation, then wringing out the excess of water, then adding a deterrent material, a flash reducing compound and a stabilizer and mixing the whole together, then subjecting the mass thus formed to pressure, then seasoning then again subjecting the material to pressure until the material becomes a translucent, cohering, colloided solid, and then cutting to the proper shapes and sizes. 25 30

CHARLES R. FRANKLIN.